

April 21, 1936.

C. S. SMITH

2,038,136

COPPER-SELENIUM ALLOYS

Filed Sept. 2, 1933



Fig. 1.



Fig. 2.

INVENTOR  
Cyril Stanley Smith  
BY  
Hoover & Davis  
ATTORNEYS.

## UNITED STATES PATENT OFFICE

2,038,136

## COPPER-SELENIUM ALLOYS

Cyril Stanley Smith, Cheshire, Conn., assignor to  
The American Brass Company, Waterbury,  
Conn., a corporation of Connecticut

Application September 2, 1933, Serial No. 687,967

10 Claims. (Cl. 75—153)

My invention concerns a series of alloys of copper distinguished by a remarkable ease of machining. The free cutting properties are achieved without great sacrifice of strength or 5 ductility by additions of selenium to pure copper or to a number of copper base alloys containing other elements. In many cases the other elements of the sulphur family, i. e., sulphur and tellurium, can be used in combination with selenium.

In the drawing:

Fig. 1 shows a set of curves demonstrating the ease of drilling copper alloys containing selenium; and

Fig. 2 shows the drillability of copper selenium alloys plotted against selenium content.

One of the principal objects of the refining operation as applied to the production of metallic copper from the crude matte is to remove 20 from the metal the elements of the sulphur family. Almost without exception these elements have been hitherto regarded as extremely harmful to the malleability and ductility of copper in both the hot and cold conditions, and for this 25 reason have been rigorously excluded. On account of this long-held opinion as to their deleterious effects they have not been subject to careful study in recent years and their true influence on copper has remained unknown. In 30 my researches I have found that none of these elements in reasonable amounts are harmful to the hot and cold working properties of copper and that they all render the metal particularly readily cut with edge tools and very suitable for the manufacture of parts on so-called automatic screw machines or by any customary machining 35 operations.

Selenium may be added to copper alloys either with the cold furnace charge or it may be added 40 to the molten alloy in the form of the element or as Cu<sub>2</sub>Se which is soluble in molten copper to the extent of about 4 per cent. selenium. On account of the volatility of the element and the poisonous nature of its fumes the latter method 45 is to be preferred. A eutectic is formed at a temperature of about 1065° C. containing approximately 3 per cent. selenium. Beyond 4.0 per cent further additions of selenium cause the formation of drops of Cu<sub>2</sub>Se which tend to float 50 out of the alloy during melting or solidification. Small amounts of selenium form eutectic areas filling in the spaces around the primary copper grains and the amount of eutectic increases with selenium additions. The eutectic of copper and 55 Cu<sub>2</sub>Se is very similar in microscopic appearance to the copper-copper oxide eutectic so familiar to metallurgists, and has even less effect on the hot working properties. The addition of other elements to binary copper-selenium alloys usually 60 coarsens the particles of Cu<sub>2</sub>Se in the eutectic

but, except in some special cases which will be discussed later, does not otherwise modify the structure.

Contrary to the general impression, I have found that it is possible to forge copper saturated with selenium and I have hot rolled alloys containing up to 1.5 per cent. selenium with no difficulty whatever, even using the severe reductions in a rolling mill designed for the commercial rolling of copper wire bars. Alloys containing up to this amount, and larger amounts, of selenium may be cold rolled, drawn or fabricated in any manner involving either hot or cold working with no particular precautions.

The alloys may also be used in the cast condition without fabrication. As with any copper alloy, it is advisable to melt and cast with exclusion of oxygen or with the addition of a de-oxidizing element in sufficient quantity to combine with the oxygen present in the melt or absorbed from the atmospheric air during pouring. I have used both methods to obtain castings from copper-selenium alloys and have obtained ingots with a deep shrinkage cavity, which, after feeding, were perfectly sound.

Alloys of copper containing appreciable amounts of selenium whether in the cast or fabricated condition are characterized by extremely high machinability. As is well known, copper is one of the most difficult metals to 30 machine, since its soft and tough character causes it to form long turnings which stick to the tool and absorb much power which appears as heat. The particles of Cu<sub>2</sub>Se in my alloys not only prevent the formation of a long chip, 35 which may foul the tool in certain types of machine operations, but they also lubricate the tool, prevent sticking and reduce to a minimum the power required for the cutting operation and the heat generated. At the same time the tool 40 life is considerably increased and a superior surface finish on the work obtained.

Alloys of copper which are desired to have free cutting qualities are at present made by additions of lead in amounts up to about 4 per 45 cent., but this, while favorably affecting machinability, does so at the expense of reducing the ductility, limiting the amount that the alloys can be cold rolled and entirely preventing hot rolling, at the same time rendering the alloys 50 susceptible to firecracking when annealed after cold working. Selenium additions are far more effective than lead in improving the machining qualities of the alloys and are quite without effect on the hot working properties. The alloys 55 moreover remain entirely immune from firecracking under severe conditions of strain and rapid heating.

Additions of selenium to copper have very little effect on the electrical conductivity and the alloys 60

should find considerable application in the manufacture of electrical devices where high electrical conductivity is necessary in a part which can be made on a high speed automatic screw machine or for parts such as bus bars which sometimes need considerable drilling and tapping during assembly.

The small effect on the electrical conductivity of copper is due to the fact that selenium is practically insoluble in solid copper but exists in the solid alloy in the form of globules of copper selenide. When the alloys are worked, these globules are elongated in the same manner as the piece as a whole, and after considerable extension form long thin fibres. The fibrous structure of the alloys is marked after very extensive rolling and results in rather poor properties when the metal is tested transversely to the direction of rolling, but an annealing or soaking operation enables the strings of selenide to break up into more or less rounded globules which have comparatively little effect on the ductility in any direction. Due to the lower ductility of the base metal, the poor transverse properties due to the long thin fibers of selenide are more marked in alloys containing other elements, for example, silicon, nickel or tin, in addition to the selenium than they are with pure copper-selenium alloys.

To show the erroneous nature of the common conception that selenium renders copper brittle, I have given in Table I the tensile properties and electrical conductivity of some copper-selenium alloys which were melted and cast in 3 in. diameter ingots and then hot rolled to  $\frac{3}{8}$  in. and cold drawn to  $\frac{1}{2}$  in. diameter, at which size the tests were made. The table also includes results of tests on the same alloys after annealing at  $600^{\circ}$  C. This temperature was not sufficiently high to spheroidize completely the Cu<sub>2</sub>Se fibers, and higher ductility would have resulted had the annealing been more drastic. The amount of selenium in these tests was limited to 1.5 per cent., since preliminary tests showed this to be sufficient for the purpose in view. However, selenium can be added in far larger amounts up to the limit of solubility, about 4 per cent., without destroying the ductility of copper.

TABLE I  
50 Tensile properties and electrical conductivity of cold drawn and annealed copper-selenium alloys

| 55                                                    | Alloy No. | Composition percent |          | Yield point<br>0.5% ext.<br>lbs./sq. in. | Tensile<br>strength<br>lbs./sq. in. | Elongation<br>in 1.4"<br>per cent. | Conductivity<br>I. A. C. S.<br>percent, 20° C. | 55 |
|-------------------------------------------------------|-----------|---------------------|----------|------------------------------------------|-------------------------------------|------------------------------------|------------------------------------------------|----|
|                                                       |           | Copper              | Selenium |                                          |                                     |                                    |                                                |    |
| <i>Cold drawn</i>                                     |           |                     |          |                                          |                                     |                                    |                                                |    |
| 55                                                    | 1601      | 99.990              | 0.010    | 50,700                                   | 52,100                              | 21.4                               | 99.7                                           |    |
|                                                       | 1614      | 99.88               | 0.110    | 51,200                                   | 53,200                              | 19.3                               | 98.9                                           |    |
|                                                       | 1603      | 99.71               | 0.26     | 51,600                                   | 53,000                              | 15.7                               | 98.0                                           |    |
| 60                                                    | 1607      | 99.37               | 0.48     | 50,900                                   | 53,600                              | 15.7                               | 97.4                                           |    |
|                                                       | 1606      | 99.02               | 1.01     | 49,300                                   | 53,400                              | 11.4                               | 94.4                                           |    |
|                                                       | 1609      | 98.57               | 1.44     | 52,000                                   | 54,200                              | 10.0                               | 92.0                                           |    |
| <i>Annealed 1 hour at <math>600^{\circ}</math> C.</i> |           |                     |          |                                          |                                     |                                    |                                                |    |
| 60                                                    | 1601      | 99.990              | 0.01     | 8,700                                    | 32,500                              | 60.0                               | 102.1                                          |    |
|                                                       | 1614      | 99.88               | 0.11     | 8,400                                    | 32,800                              | 57.1                               | 99.0                                           |    |
|                                                       | 1603      | 99.71               | 0.26     | 8,900                                    | 32,500                              | 55.7                               | 100.1                                          |    |
| 65                                                    | 1607      | 99.37               | 0.48     | 8,000                                    | 32,800                              | 52.9                               | 98.8                                           |    |
|                                                       | 1606      | 99.02               | 1.01     | 8,500                                    | 33,300                              | 48.6                               | 95.6                                           |    |
|                                                       | 1609      | 98.57               | 1.44     | 10,100                                   | 33,200                              | 42.1                               | 94.4                                           |    |

These alloys were hot rolled from 3 in. to 0.625 in., annealed and cold drawn to 0.5 in. in one pass. Gauge length of test pieces—0.357 in. diameter.

To demonstrate the remarkable ease of machining the alloys, I have reproduced in Figure 1 the results of some crude drill tests. These curves

show the number of turns necessary for a drill 0.25 in. diameter to penetrate 0.25 in. into the metal under the load shown. For comparison, a leaded brass containing 3 per cent. lead and 35 per cent. zinc was included in the tests as shown by dotted curve A, together with pure copper as shown by curve B.

It will be seen that the alloys containing as little as 0.1 per cent. selenium are much easier to drill than pure copper, and that successive additions up to 1.5 per cent. progressively increase the amount of metal removed at each turn of the drill, although the improvement is not proportionally as great above 0.5 per cent. selenium as below this. The alloys containing 0.5 per cent. selenium are about equal in behavior to the leaded brass, while with more selenium than this the alloys are superior.

An improvement in machinability is secured with any addition of selenium as shown in Fig. 2 but to secure a material improvement selenium should be added in amount from approximately 0.05 per cent. up to the limit of solubility which is approximately 4.0 per cent., but the preferred range is from approximately 0.25 per cent. to 1.0 per cent.

The addition of selenium according to my invention is not limited to pure copper alone. I have found that the selenium additions may be satisfactorily made and the improvement in the machinability obtained without severe loss of ductility when copper is also alloyed, for example, with silicon, tin, nickel and/or zinc. The copper base alloys containing silicon or tin are strong and corrosion resistant, while those containing nickel are attractive on account of their white color and their resistance to tarnish and corrosion.

In the case of copper-nickel alloys of high nickel content, for example 70 per cent. nickel, there is apparently formed a low melting point constituent or eutectic containing nickel and selenium which interferes seriously with the malleability of the alloys. The amount of nickel that can be tolerated without the formation of this brittle constituent can be increased by the addition of zinc, but alloys containing up to approxi-

mately 30 per cent. nickel and 1.0 per cent. selenium are malleable both hot and cold in the absence of zinc. Alloys of somewhat higher nickel content are malleable if the selenium content is reduced.

Additions of zinc to alloys containing copper, nickel and selenium improve the casting and

bricating properties, and the alloys containing in the range of 10 to 30 per cent. nickel with 0.1 to 10 per cent. zinc and 0.05 to 2.0 per cent. selenium would be preferred for general use. If zinc is added in excess of approximately 10 per cent. it commences to form a zinc selenide which is not completely soluble in the molten alloy and commences to segregate. However, with smaller amounts of zinc this does not happen and the zinc selenide, if formed, apparently remains in solution in the Cu<sub>2</sub>Se inclusions or is associated with them forming duplex inclusions which do not separate in the liquid state. Additions of tin in amount of approximately 1 per cent. also improve the malleability of the alloys of copper with nickel and selenium and increase the amount of nickel that could be present without embrittlement occurring.

The alloys of copper and tin have found application since prehistoric times where a strong corrosion resisting alloy was required. The amount of tin is usually not over 11.0 per cent. where the alloys are to be cold rolled, but may be as high as 18 per cent. in alloys which are used in the cast condition. Usually to improve the casting qualities a small amount of phosphorus, silicon or zinc is added to the alloys. I have found that selenium in appreciable amounts and up to 1.5 per cent. may be added to bronzes containing appreciable amounts of tin and up to 18 per cent. and confers great machinability without rendering the alloys brittle. Alloys of copper with tin and selenium with a suitable deoxidizer make satisfactory sand castings. Chill castings, die castings, or permanent mold castings, can also be made from the alloys containing selenium.

Copper alloys with silicon in all proportion, but there is useful ductility only in the range up to approximately 5 per cent. silicon. These alloys find considerable application in industry, usually in combination with some other element to improve the strength or otherwise modify the properties. I have studied alloys of copper containing approximately 4 per cent. silicon and various amounts of selenium up to 1.0 per cent. and have found the properties to be as shown in Table II. Table II also includes a "machinability index", corresponding to the number of turns of a 0.25 in. drill to penetrate 0.25 in. into the alloy under a load of 86 pounds. The addition of selenium will be seen to increase the machinability and to have comparatively small effect on the strength and ductility.

These alloys were hot rolled from 3 in. to 0.625 in., annealed and cold drawn to 0.5 in. in two passes. Gauge length of test pieces—0.357 in. diameter.

Although it does not seem possible to add selenium to the brasses of high zinc content, selenium may be added to copper-zinc alloys containing up to 15 or 20 per cent. zinc and a great improvement in machinability obtained.

The group of alloys containing in addition to copper and selenium also silicon, or tin, or nickel, or zinc, or a combination of copper and selenium with tin or nickel and zinc were selected and studied as representing important groups of copper alloys at present finding application. Most of these alloys as commercially produced contain also additional elements which serve to improve the properties in various ways and new copper alloys will undoubtedly be developed in the future based on these or entirely new combination of elements. Selenium may be added to any complex copper alloys with as much facility as to the binary alloys unless there is present a large amount of some element which combines with selenium and forms a selenide which is not soluble in the liquid alloy. When this occurs selenium is rapidly eliminated and does not remain evenly distributed throughout the casting. Among the common elements which do not prevent the retention of selenium in the alloy, I have found the following: Fe, Sn, Sb, Ag, P, Cd, Si, Ni, while the elements Al, Mg, Ca, Zr, and Mn if present in more than a small quantity tend to eliminate the selenium, while zinc if present in more than perhaps 15 per cent. has a similar effect. In the case of manganese, amounts up to 0.5 per cent. are permissible, although 1.0 per cent. causes segregation of selenium. For all those elements which combine with selenium more avidly than does copper, there will be a limiting concentration below which the insoluble selenide will not form and the selenium will remain distributed uniformly throughout the alloy, but above which concentration the selenide is insoluble in the liquid state.

Although I have disclosed herein the addition of selenium to copper and a few specific alloys, it is at once obvious that the addition may be made to any alloys of copper with the disclosed or other elements, singly or combined in any manner, providing there is not an excessive

TABLE II  
55 Tensile properties and machinability of cold drawn and annealed copper-silicon alloys containing selenium

55

| 60                                | Alloy No. | Composition percent |                    | Yield point<br>0.5% ext.<br>lbs./sq. in. | Tensile strength<br>lbs./sq. in. | Elongation<br>in 1.4" per-<br>cent | Reduction of<br>area percent | Machin-<br>ability index* | 60 |
|-----------------------------------|-----------|---------------------|--------------------|------------------------------------------|----------------------------------|------------------------------------|------------------------------|---------------------------|----|
|                                   |           | Silicon             | Selenium           |                                          |                                  |                                    |                              |                           |    |
| <i>Cold drawn</i>                 |           |                     |                    |                                          |                                  |                                    |                              |                           |    |
| 65                                | 1626      | 3.70                | 0.0                | 55,800                                   | 111,850                          | 16.4                               | 56.0                         | (320)                     |    |
|                                   | 1630      | 3.83                | 0.12               | 55,750                                   | 113,250                          | 16.4                               | 54.5                         | 164                       | 65 |
|                                   | 1629      | 3.86                | 0.25               | 54,700                                   | 112,100                          | 15.0                               | 48.1                         | 103                       |    |
|                                   | 1628      | 3.82                | 0.51               | 52,900                                   | 110,300                          | 10.0                               | 29.8                         | 89                        |    |
|                                   | 1627      | 3.85                | 0.98               | 49,250                                   | 109,750                          | 9.3                                | 16.4                         | 77                        |    |
|                                   | 1633      | 3.76                | { 0.25+<br>0.24% S | 51,450                                   | 111,750                          | 9.3                                | 23.4                         | 93                        |    |
| <i>Annealed 1 hour at 750° C.</i> |           |                     |                    |                                          |                                  |                                    |                              |                           |    |
| 70                                | 1626      | 3.79                | 0.0                | 20,400                                   | 61,050                           | 70.7                               | 67.8                         | (192)                     |    |
|                                   | 1630      | 3.83                | 0.12               | 23,300                                   | 62,550                           | 67.1                               | 70.3                         | 196                       | 70 |
|                                   | 1629      | 3.86                | 0.25               | 25,550                                   | 62,850                           | 64.7                               | 66.6                         | 114                       |    |
|                                   | 1628      | 3.82                | 0.51               | 26,250                                   | 61,500                           | 59.3                               | 47.8                         | 85                        |    |
|                                   | 1627      | 3.85                | 0.98               | 29,000                                   | 61,900                           | 49.7                               | 36.7                         | 77                        |    |
|                                   | 1633      | 3.76                | { 0.25+<br>0.24% S | 29,000                                   | 62,100                           | 53.6                               | 43.1                         | 87                        |    |

\* Number of turns of 0.25 in. drill necessary to penetrate 0.25 in. under load of 86 pounds.

amount of selenide formed that is insoluble in the liquid alloy and that is sufficiently different in density to be rapidly eliminated from the molten alloys. As examples of complex alloys I have made and used those containing copper with silicon, tin and selenium; copper with silicon, iron, zinc and selenium; copper with nickel, zinc and selenium; copper with nickel, zinc, tin and selenium; copper with tin, zinc and selenium. It is obvious, however, that there is almost no limit to the alloys of copper which can be made and to which selenium is a helpful addition when free-cutting qualities are desired. My invention covers the addition of selenium either as the element, copper-selenide or any other form to relatively pure copper or to any alloys of copper from which the selenium is not eliminated during casting.

Some of the alloys with selenium which are of importance include the following:

An alloy containing selenium from 0.05 to 4.0 per cent. the balance being substantially copper.

An alloy containing selenium approximately 1.0 per cent. and copper approximately 99.0 per cent.

An alloy consisting of approximately 0.5 per cent. selenium and 99.5 per cent. copper.

Alloys containing from 0.05 per cent. to 4.0 per cent. selenium, the balance being principally copper with additions of one or more of the following: 0 to 5 per cent. silicon, 0 to 20 per cent. zinc, 0 to 50 per cent. nickel, 0 to 5 per cent. iron, 0 to 15 per cent. tin, 0 to 2 per cent. cadmium.

An alloy containing 0 to 5 per cent. silicon, 0.05 to 2 per cent. selenium, and 93 to 99.5 per cent. copper.

An alloy containing approximately 4.0 per cent. silicon, approximately 1.0 per cent. selenium, and approximately 95.0 per cent. copper.

Alloys containing 0 to 5 per cent. Si, 0 to 11 per cent. Fe, 0 to 10 per cent. Zn, 0.05 to 2 per cent. Se, and the balance being principally copper.

An alloy containing approximately 3.5 per cent. Si, 2 per cent. Fe, 2 per cent. Zn, 1 per cent. Se, the balance being principally copper.

Alloys containing 0 to 5 per cent. Si, 0 to 10 per cent. Sn, 0.05 to 2 per cent. Se, the balance being principally copper.

An alloy containing approximately 1.75 per cent. Si, 1.0 per cent. Sn, 1.0 per cent. Se, the balance being principally copper.

Alloys containing 0 to 30 per cent. Ni, 0.05 to 2 per cent. Se, and the balance being principally copper.

An alloy containing approximately 20.0 per cent. Ni, 1.0 per cent. Se, the balance being principally copper.

Alloys containing 0 to 50 per cent. Ni, 0 to 15 per cent. Zn, 0.05 to 2.0 per cent. Se, the balance being principally copper.

An alloy containing approximately 20 per cent. Ni, 5 per cent. Zn, 1.0 per cent. Se, the balance being principally copper.

Alloys containing 0 to 15 per cent. Sn, 0.05 per cent. to 2.0 per cent. Se, the balance being principally copper.

An alloy containing approximately 5.0 per cent. Sn, 1.0 per cent. Se, the balance being principally copper.

An alloy containing approximately 5.0 per cent. Sn, 1.0 per cent. Zn, 1.0 per cent. Se, the balance being principally copper.

Alloys containing 0 to 20 per cent. Zn, 0.05 to

2.0 per cent. Se, the balance being principally copper.

An alloy containing approximately 10 per cent. Zn, 1 per cent. Se, the balance being principally copper.

Alloys containing 0 to 50 per cent. nickel, 0 to 4 per cent. tin, 0.05 to 2.0 per cent. selenium, the balance being principally copper.

An alloy containing approximately 30 per cent. nickel, 1.0 per cent. tin, 1.0 per cent. selenium, 10 the balance being principally copper.

Alloys containing 0 to 5 per cent. silicon, 0 to 10 per cent. zinc, 0 to 5 per cent. tin, 0.05 to 2.0 per cent. selenium, the balance being principally copper.

An alloy containing approximately 3.25 per cent. silicon, 1.5 per cent. zinc, 0.5 per cent. tin, 1.0 per cent. selenium, the balance being principally copper.

The other elements of the sulphur family, viz., sulphur and tellurium, behave in a manner similar to selenium. It may prove advisable to use additions of two or more of these elements simultaneously and it should be understood that whenever selenium is mentioned in this specification, selenium with more or less of the elements sulphur or tellurium, or sulphur and tellurium may be included.

It is possible to add selenium or a suitable selenide to alloys made by the process of compressing powders and sintering at a temperature below the melting point. In this case there is no limit to the alloys with which selenium can be combined, for the lack of solubility in the liquid state is of no importance.

The lubricating nature of the copper selenide as shown by its action on the cutting tool suggests that the alloys containing selenides would be useful for bearing purposes.

Having thus set forth the nature of my invention, what I claim is:

1. An alloy containing selenium from 0.1 per cent. to 4.0 per cent., the balance being copper.

2. An alloy containing from approximately 0.25 per cent. to 1.0 per cent. selenium, the balance being copper.

3. An alloy containing selenium approximately 1.0 per cent. and copper approximately 99.0 per cent.

4. An alloy consisting of approximately 0.5 per cent. selenium, and approximately 99.5 per cent. copper.

5. A substantially zinc free copper base alloy 55 which is characterized by ease of machining and which is workable by hot or cold rolling containing selenium in amount from 0.1 per cent. to 4.0 per cent.

6. A substantially zinc free copper base alloy 60 which is characterized by ease of machining and which is workable by hot or cold rolling containing selenium in amount from approximately 0.25 per cent. to approximately 1.0 per cent.

7. A substantially zinc free copper base alloy 65 which is characterized by ease of machining and which is workable by hot or cold rolling containing approximately 0.5 per cent. selenium.

8. A copper base alloy other than a brass of over 15 per cent. zinc which is characterized by ease of machining and which is workable by hot or cold rolling containing selenium in amount from 0.1 per cent. to 4.0 per cent.

9. A copper base alloy other than a brass of 75

over 15 per cent. zinc which is characterized by ease of machining and which is workable by hot or cold rolling containing selenium in amount from approximately 0.25 per cent. to approximately 1.0 per cent.

5 10. A copper base alloy other than a brass of

over 15 per cent. zinc which is characterized by ease of machining and which is workable by hot or cold rolling containing approximately 0.5 per cent. selenium.

CYRIL STANLEY SMITH. 5